

# United States Patent [19]

Arnold

[11]

4,299,64

[45]

Nov. 10, 198

[54] HEAT TRANSFER DECAL

[75] Inventor: **Raymond M. Arnold**, West Chester, Pa.

[73] Assignee: **Advanced Graphic Technology**, Chicago, Ill.

[21] Appl. No.: 73,554

[22] Filed: **Sep. 6, 1979**

[51] Int. Cl.<sup>3</sup> ..... **B44C 1/24**

[52] U.S. Cl. ..... **156/230; 156/277; 260/33.4 R; 260/33.2 R; 260/31.2 R; 427/407.1; 427/411**

[58] Field of Search ..... **260/33.4 R, 33.2 R, 260/31.2 R; 427/407.1, 411; 156/230, 277**

[56]

References Cited

U.S. PATENT DOCUMENTS

|           |         |          |            |
|-----------|---------|----------|------------|
| 3,764,587 | 10/1973 | Zunker   | 260/33.8 U |
| 3,919,150 | 11/1975 | Kiel     | 260/33.2   |
| 4,136,076 | 1/1979  | Daniels  | 260/33.4   |
| 4,138,522 | 2/1979  | Ishizuka | 260/33.2   |
| 4,177,076 | 12/1979 | Sato     | 260/33.4   |

Primary Examiner—Paul R. Michl

Attorney, Agent, or Firm—Allegretti, Newitt, Witcoff  
McAndrews

[57]

ABSTRACT

A method for producing a multicolor heat transfer decal comprises printing specially formulated thermoplastic inks successively onto a pre-release coated carrier sheet. The inks give optimum print quality using plastic printing plates and a rotary letterpress or flexographic printing process.

7 Claims, 1 Drawing Figure





## HEAT TRANSFER DECAL

## BACKGROUND OF THE INVENTION

This invention relates to multicolor heat transfer decals particularly as used to decorate plastic articles.

In order to produce heat transfers that give high quality images and show clear and brilliant colors, a screen process (e.g. silk screen) was originally used. The screen process enabled a printer to formulate inks that were compatible with the various plastics to be decorated since there were virtually no restrictions on the solvents that could be used to dissolve the resins that were needed to make the inks. Screen process inks are conventionally made using slow drying solvents such as white spirit, high boiling aromatics, ketones and glycol ethers.

To satisfy a larger volume market for heat transfers that could not be met by the comparatively slow silk screen process, various methods were devised using a gravure printing process. Gravure printing has the advantage that almost any solvent system can be used due to the solvent impervious etched metal rollers that are used to carry out gravure printing. For example, very fast evaporating solvents such as toluene, methyl ethyl ketone and N-propyl acetate are used.

Many of the gravure heat transfer systems employ an adhesive layer or a wax to bond conventional printing inks down onto the final receptor surface or carrier film. U.S. Pat. Nos. 2,862,332 and 2,989,413 disclose examples of such a wax bonding system. The wax acts as a release system and as a bonding agent.

Other systems have a release layer similar to that used in the foil stamping industry. Such release layers are commonly mixtures of waxes and a high molecular weight acrylic. The inks associated with such systems are based on resins that are only soluble in very active solvents.

There are serious disadvantages in using either silk screen process or gravure process. The screen process is very slow and requires new screens each time a particular design is run since the screens are very susceptible to damage. With such processes, very fine color process printing beyond 60-80 lines per inch is difficult thereby seriously limiting the quality of work that can be produced. The nature of the processes preclude close registration of printed material.

Since heat transfers are generally required in a roll or web format, screen printing machines having the ability to print on web form have been developed. However, they are very costly and require highly trained operating personnel.

The gravure process is ideal for producing high quality heat transfers. Thermoplastic inks printed over release coated film give the finest print quality. However, this too is a very costly process. The printing equipment is very expensive and the costs of preparing gravure cylinders is extremely high since highly skilled personnel are necessary for their manufacture. A gravure processing plant has a high capital cost further escalating the cost.

Alternative processes have been proposed. Various early heat transfers were printed using rubber plates on conventional flexographic equipment. However, the rubber plates give very poor quality reproduction and the inks used are not thermoplastic. Also, a secondary adhesive coating must be applied to give adhesion to the articles being decorated. The colors are very weak and

tend to be transparent and have very poor resistance to abrasion. Consequently, this early process was discontinued.

In recent times the invention of plates made from photopolymer resins such as Dupont Cyrel® resin and BASF Nyloprint® resin plates has resulted in a high quality plate that can give resolution and definition in letterpress printing much closer to that achieved by the gravure process. The solvent system that can be used with these "plastic" plates, however, is still similar to that used with the older rubber printing plates although the plastic plates will tolerate a higher percentage of more active solvent in the inks. Commonly used solvents therefore consist mainly of ethanol or isopropanol with additions in the order of 10% of propyl acetate, nitropropane and glycol ethers.

## SUMMARY OF THE INVENTION

The present invention comprises the discovery of inks and their use to provide required heat transfer characteristics when printed on heat activated release coated material such as wax or resin coated polyester film or polymer coated paper e.g. polypropylene or kraft paper. The inks can be printed using the "plastic" printing plates and result in a method of producing heat transfers that eliminate the disadvantages of the prior art gravure or screen processes. The resultant product is a very high quality heat transfer product having a competitive cost.

The machines used to print the heat transfers are conventional rotary letterpress or flexographic presses which are commonly available and which have a much lower capital cost than either web fed gravure presses or web screen presses. Such presses can also be operated by their normal operators. The plastic printing plates also can be readily made using conventional processing equipment and normal personnel. The cost of such plates is only a fraction of the cost of gravure cylinder. Such plates also have the added advantage of being readily stored for use with subsequent orders.

In order to utilize the ease of print that the flexographic process offers and yet obtain the resistance to solvent and adhesion of more difficult to decorate surfaces, it is possible to utilize a combination gravure and plastic plate, flexographic process. For example, a gravure unit may be used for the first step to deposit a release coating. If the substrate or carrier film is already release coated (as is the normal case) another protective coating gives added abrasion or solvent resistance. Upon transference this first applied coating becomes the uppermost layer. Also, use of a gravure unit after heat transfer inks are laid down over the release coating allows the application of tie coats to give improved adhesion to difficult surfaces. In both of these gravure steps the coating would be continuous over the whole surface and not in register with the ink design element. This would permit utilization of simple coating rollers that could be used with all and any designs.

Thus it is an object of the present invention to provide an improved method of printing heat transfers by means of inexpensive flexographic processes using inexpensive flexographic plates.

A further object of the present invention is to provide improved heat transfer ink formulations which may be used for various printing processes for the manufacture of heat transfer decals.

Still another object of the present invention is to provide a method of manufacture of a heat transfer from carrier film particularly to a plastic surface wherein the transfer has high abrasion resistance and durability.

Another object of the present invention is to provide an inexpensive method for manufacture of heat transfers using currently available printing equipment in combination with new and specific formulations of heat transfer ink.

These and other objects, advantages and features of the invention will be set forth in the detailed description which follows.

#### BRIEF DESCRIPTION OF THE DRAWING

The drawing comprises a single FIGURE illustrating schematically the various steps in the method of the present invention.

#### DESCRIPTION OF THE PREFERRED EMBODIMENT

Generally, with the present invention, a carrier film or substrate is provided for the heat transfer. Heat transfer inks are then printed on the carrier film by means of known flexographic or letter press methods. Prior to printing of the heat transfer ink on the film, a coating may be applied to the film to improve abrasion resistance of the ultimate heat transfer. The coating thus is of a type which would be released from the film by the heat transfer operation.

Subsequent to printing of formulated inks upon the film, it is also an optional step of the invention to apply a coating of tying material or adhesion promotion material. The application of the pre and post ink materials may be by gravure methods or by any other suitable printing method. The inks, however, are generally applied by flexographic or letterpress methods. The sequence of operations is illustrated in the drawing.

Preferably the plates used for the letter press or flexographic printing of the transfer inks are plastic plates which provide for high resolution printing. Typical plastic plates include those made from photopolymer resins such as the tradename products Cyrel by Dupont and Nyloprint by BASF.

Preferably the general composition of the printing inks is as follows:

Organic pigment or dye: 1-30% by weight  
 Alcohol solution acrylic resin: 3-12% by weight  
 Cellulose acetate butyrate: 0.5-5% by weight  
 Dispersion agents: 0.0-2% by weight  
 Ethanol (solvent): 25-50% by weight  
 Butyl cellosolve (solvent): 5-12% by weight  
 \*Pentoxone (solvent): 0.0-3% by weight  
 2-Nitro propane (solvent): 10-25% by weight  
 N-propyl acetate (solvent): 5-15% by weight  
 Registered trademark of Shell Chemical Company-4 methoxy 4 nethyl pentanone-2 (solvent).

The following examples give various examples of combinations of carriers, printing inks, tie down materials and release materials which may be used in the printing process.

#### EXAMPLE 1

A roll of polyester film 0.001" in thickness was precoated with a release coating as follows:

\*Elvacite 2041—15%  
 Toluene—40%  
 Methyl ethyl ketone—35%  
 A high molecular weight acrylic resin supplied by Dupont Co.

This coating is applied by gravure or metering bar process to give a dry coating weight of 0.2 grams per square meter.

Inks can be printed over this layer. The inks typically have the following formulations:

|    | (1) BLUE INK                | Supplier       | Percentage by Weight |
|----|-----------------------------|----------------|----------------------|
| 10 | Phthalocyanene blue pigment | Dupont         | 7.70 ± 3.00          |
|    | Orasol solvent soluble dye  | Ciba Geigy     | 4.20 ± 2.00          |
|    | Titanium dioxide            | Dupont         | 1.40 ± 1.00          |
|    | <sup>1</sup> Elvacite 2013  | Dupont         | 9.23 ± 3.00          |
| 15 | Cellulose acetate butyrate  | Eastman Kodak  | 2.28 ± 1.50          |
|    | <sup>2</sup> Span 80        | I.C.I.         | .04 ± .02            |
|    | <sup>3</sup> G. 3300        | I.C.I.         | .04 ± .02            |
|    | Ethanol                     |                | 34.17 ± 5.00         |
|    | Pentoxone                   | Shell Chemical | .71 ± 1.50           |
|    | Butyl cellosolve            |                | 8.02 ± 2.50          |
| 20 | <sup>4</sup> Paraplex G. 60 | Rohm and Haas  | 3.49 ± 1.75          |
|    | 2. Nitro propane            |                | 19.42 ± 5.00         |
|    | N-propyl acetate            |                | 9.30 ± 5.00          |
|    |                             |                | 100.00%              |

<sup>1</sup>Elvacite 2013 - a low molecular weight methyl/n butyl methacrylate copolymer resin

<sup>2</sup>Span 80 - sorbitan mono oleate, wetting agent

<sup>3</sup>G. 3300 - ionic surfactant - alkyl aryl sulphonate, dispersant

<sup>4</sup>Paraplex G. 60 - a polymeric plasticizer

|    | (2) YELLOW INK                             | Supplier       | Percentage by Weight |
|----|--------------------------------------------|----------------|----------------------|
| 30 | Dalamar yellow pigment                     | Dupont         | 4.99 ± 5.00          |
|    | Orasol yellow 2 gln. dye                   | Ciba Geigy     | 3.00 ± 2.00          |
|    | Titanium dioxide                           | Dupont         | 1.46 ± 1.00          |
|    | Elvacite 2013                              | Dupont         | 10.62 ± 3.00         |
| 35 | Cellulose acetate butyrate                 |                | 2.64 ± 1.50          |
|    | Span 80 (sorbitan olate)                   | I.C.I.         | .18 ± .10            |
|    | G. 3300 (Alkyl aryl sulphonate)            | I.C.I.         | .18 ± .10            |
|    | Ethanol                                    |                | 34.46 ± 5.00         |
|    | Pentoxone (4-Methoxy 4-Methyl Pentanone-2) | Shell Chemical | 1.93 ± 1.50          |
| 40 | Butyl cellosolve                           |                | 5.49 ± 2.50          |
|    | N-propyl acetate                           |                | 12.70 ± 5.00         |
|    | Paraplex G. 60 (polymeric plasticizer)     | Rohm and Haas  | 2.40 ± 1.75          |
|    | 2. Nitro propane                           |                | 19.95 ± 5.00         |
|    |                                            |                | 100.00%              |

|    | (3) WHITE INK                             | Supplier       | Percentage by Weight |
|----|-------------------------------------------|----------------|----------------------|
| 50 | Titanium dioxide                          | Dupont         | 29.88 ± 7.50         |
|    | Elvacite 2013 (Methyl Butyl Methacrylate) | Dupont         | 9.50 ± 3.00          |
|    | Cellulose acetate butyrate                |                | 2.29 ± 1.50          |
|    | 2. nitro propane                          |                | 13.40 ± 5.00         |
| 55 | Butyl cellosolve                          |                | 5.24 ± 2.50          |
|    | Ethanol                                   |                | 28.72 ± 5.00         |
|    | N-propyl acetate                          |                | 7.05 ± 5.00          |
|    | Span 80                                   | I.C.I.         | .06 ± .10            |
|    | G. 3300                                   | I.C.I.         | .06 ± .10            |
| 60 | Pentoxone                                 | Shell Chemical | 1.51 ± 1.50          |
|    | Paraplex G.60                             | Rohm and Haas  | 2.29 ± 1.75          |
|    |                                           |                | 100.00%              |

The inks were printed using Dupont Cyrel photopolymer plates. On the application of heat and pressure the inks transferred cleanly and easily to an article made of high impact polystyrene giving a decoration with excellent abrasion resistance.

## EXAMPLE 2

A coating consisting of Ouricury wax dissolved as a 5% solution in trichlorethylene was applied to 0.00075 polyester carrier film using a wire wound metering bar and inks as described in Example 1 above were printed using B.A.S.F. Nyloprint photopolymer or plastic plates.

The resultant print transferred easily and cleanly on application of heat and pressure to a plastic article made of polycarbonate resin.

## EXAMPLE 3

A coating of Ouricury wax on polyester film as described in Example 2 was overcoated with the following abrasion resistant lacquer:

|                                               | Supplier         | Percentage by Weight |
|-----------------------------------------------|------------------|----------------------|
| <sup>1</sup> V.Y.H.H.                         | Bakelite         | 3.30 ±               |
| <sup>2</sup> Acryloid A.101<br>(30% solution) | Rohm and Haas    | 13.00 ±              |
| <sup>3</sup> Chlorowax 40                     | Diamond Shamrock | 2.70 ±               |
| Methyl ethyl ketone                           |                  | 40.00 ±              |
| Toluene                                       |                  | 41.00 ±              |
|                                               |                  | 100.00%              |

<sup>1</sup>V.Y.H.H. - medium molecular weight vinyl chloride-vinyl acetate copolymer

<sup>2</sup>Acryloid A.101 - high molecular weight methyl methacrylate

<sup>3</sup>Chlorowax 40 - chlorinated paraffin wax

The coating was applied by wire wound metering bar giving a dry coating weight of 2-5 grams per square meter.

The duplex coated film was then printed on the flexographic press using Cyrel plates with the inks as described in Example 1.

The resultant multi-layer system, when applied by use of heat and pressure to polystyrene, resulted in a 35 hard, abrasion and alcohol resistant decoration suitable for decorating cosmetic containers.

## EXAMPLE 4

An overall key or tie coating was applied by using a 40 plain Cyrel (Dupont) plate. The coating had the following formulation and was applied over previously inked film as described in above examples:

|                             | Supplier      | Percentage by Weight |
|-----------------------------|---------------|----------------------|
| CP. 515-2                   |               |                      |
| Chlorinated polyolefin      | Eastman Kodak | 39.00 ± 7.50         |
| Elvax 40 (10% in heptane)   |               |                      |
| Ethylene vinyl acetate      | Dupont        | 18.96 ± 5.00         |
| Aerosil 300 (Silica filler) | Degussa       | 4.37 ± 7.00          |
| Heptane (solvent)           |               | 37.67 ± 10.00        |
|                             |               | 100.00%              |

This system gave good adhesion to polyethylene and polypropylene when transferred using heat and pressure.

## EXAMPLE 5

Inks based on the following formulations were printed from Cyrel (Dupont) plastic printing plates onto release coated polyester film.

|                                                     | Supplier               | Percentage By Weight | Range  |
|-----------------------------------------------------|------------------------|----------------------|--------|
| <sup>1</sup> Krumbhaar Resin 1717<br>(50% solution) | Lawter<br>Chemical Co. | 30.00                | 20-30% |
| Precipitated<br>chalk (pigment)                     |                        | 21.00                | 5-25%  |

## -continued

|                                             | Supplier      | Percentage By Weight | Range    |
|---------------------------------------------|---------------|----------------------|----------|
| <sup>2</sup> Versamid 750<br>(40% solution) | General Mills | 15.00                | 10-20%   |
| Dye                                         |               | 4.00                 | 0-7%     |
| N-propyl acetate<br>(solvent)               |               | 11.00                | 5-15%    |
| Nitrocellulose<br>(½ sel grade)             | Hercules      | 15.00                | 2-7%     |
| Di-octyl phthalate<br>plasticizer           |               | 2.00                 | 0.5-3.5% |
| Titanium dioxide                            |               | 1.80                 | 0-7%     |
| Dispersion agents                           |               | 0.20                 | 0-2%     |
|                                             |               | 100.00%              |          |

<sup>1</sup>Krumbhaar Resin 1717 - condensed ketone resin

<sup>2</sup>Versamid 750 - polyamide resin

On application of heat and pressure these inks will out any further tie coat or adhesion promoter will adhere to low and high density polyethylene and polypropylene.

In the examples, various ranges of constituents have been set forth. Additionally, alternative components have been identified.

While there has been set forth various preferred embodiments of the method and formulations associated with the present invention, it is to be understood, however, that various changes can be made while not departing from the spirit and scope of the invention. The invention is to be limited only by the following claims and their equivalents.

What is claimed is:

1. A method for manufacture of heat transfer decal comprising the steps of:

(a) providing a release coated carrier film from the group consisting of polypropylene coated paper, cured melamine coated paper, epoxy coated paper and polyester film; and

(b) printing on said film by means of flexographic methods with at least one ink from a group of inks having the following formulation:

Pigment or dye: 1-30% by weight

Alcohol solution acrylic resin: 3-12% by weight

Cellulose acetate butyrate: 0.5-5% by weight

Dispersion agents: 0.0-2% by weight

Ethanol: 25-50% by weight

Butyl cellosolve: 5-12% by weight

4. Methoxy-4 Methyl, Pentanone-2: 0.0-3% by weight

2-Nitro propane: 10-25% by weight

N-propyl acetate: 5-15% by weight

Polymeric plasticiser: 1-5% by weight.

2. The method of claim 1 including the additional step of subsequently overcoating the printed inks with a tie coat to promote added adhesion of said heat transfer decal to a surface.

3. The method of claim 1 including the addition of a preliminary step of applying a precoat from the group consisting of hard acrylic and resin to the film prior to printing the ink on the film to provide added abrasion and solvent resistance for the heat transfer.

4. The method of claim 1 comprising the step of printing said ink on the film by means of photopolymer plastic printing plates.

5. The method of claim 1 comprising the step of providing a polyester carrier film with a coating from the group consisting of wax and resin.

6. The method of claim 5 including the additional step of subsequently transferring the transfer by heat and pressure onto polyolefinic plastic material.

7. The method of claim 1 including the step of providing a release substrate from the group consisting of silicone and organic chromium complex for the carrier film.

\* \* \* \* \*